

Feb. 23, 1926.

1,573,963

A. ISAACS

DUPLICATING ROLL OR SHEET AND PROCESS OF MAKING SAME

Original Filed May 5, 1923

Fig-1



Fig-2



Albert Isaacs Inventor:  
By his Attorney  
Edmund Congan Brown

## UNITED STATES PATENT OFFICE.

ALBERT ISAACS, OF NEW YORK, N. Y., ASSIGNOR TO THE BECK DUPLICATOR COMPANY, A CORPORATION OF NEW YORK.

## DUPLICATING ROLL OR SHEET AND PROCESS OF MAKING SAME.

Application filed May 5, 1923, Serial No. 636,970. Renewed August 29, 1925.

To all whom it may concern:

Be it known that I, ALBERT ISAACS, a citizen of the United States, and a resident of the borough of Queens, city and State of New York, have invented certain new and useful Improvements in Duplicating Rolls or Sheets and Processes of Making Same, of which the following is a specification.

My invention relates to duplicating rolls 10 or sheets for duplicating machines and to the processes by which the same are made, and more particularly to an improved form of roll or sheet and to the processes by which the same is made and by which the duplicating medium forming a part of the said roll is quickly, easily and securely attached to the foundation or backing of the roll.

The invention consists in the new and improved process by which such a roll or sheet 20 is produced, and in the roll or sheet produced by the said process, all as set forth in the claims forming part of this specification, one form or embodiment thereof being described in this specification, and a roll or 25 sheet made in accordance therewith shown in the accompanying drawings.

In the said drawings,

Fig. 1 is a perspective view of a portion 30 of a roll or sheet made according to my improved process and embodying my invention; and

Fig. 2 is a vertical section through such a roll or sheet.

In the manufacture of duplicating rolls 35 or sheets, one of the difficulties which is encountered is that of causing the duplicating material, which is usually a hot gelatinous composition, to adhere to the backing or foundation of the roll or sheet. This backing or foundation may be paper or may be a woven fabric, sometimes coated on one side, as oilcloth or the like. The gelatinous composition is applied to the base or foundation 40 by pouring the same on in a liquid heated state, with or without the interposition of some suitable substance which may be waterproof, glycerine-proof, or the like, as is desired by the manufacturer to meet particular conditions.

For various reasons, the gelatinous composition does not always adhere to the base 50 or foundation when it is poured directly thereon, nor has there yet been found any entirely satisfactory material with which the foundation may be coated for the pur-

pose of giving greater adherence to the duplicating composition. The substances used for this purpose have been in the nature of drying oils or paints or the like, which, after 60 hardening by the oxidizing action of the air, are not appreciably softened by heat or other means. I have found that by interposing between the backing and the gelatinous composition a material which is liquefied or softened by a less degree of heat than 65 that which is required to reduce to a suitable pouring condition the gelatinous composition, and then pouring the liquid heated gelatinous composition thereupon and allowing both to cool and harden together, an 70 entirely satisfactory adhesion and union of the three elements of the roll or sheet, namely, the backing, the adhesive substance, and the gelatinous composition, is produced.

In carrying my invention into effect 75 in the particular embodiment thereof which I here describe, I provide a sheet of backing or foundation material, which may be of any suitable material and of any desired length, and I coat one side of the same 80 with some suitable material in the melting point of which is in the neighborhood of one hundred to one hundred and ten degrees Fahrenheit. I have found in practice that a suitable rubber cement, or the material 85 which is known in the trade as balatan, is satisfactory for this purpose. The same may be applied in any suitable manner as will be well understood by those skilled in the art. After this layer of adhesive material has 90 become solidified I pour thereon the hot liquid gelatinous composition. This composition usually has a melting point of about one hundred and fifty degrees Fahrenheit, consequently, when it is poured up- 95 on the previously applied adhesive coating, the heat of the gelatine partially melts or liquifies the adhesive coating before the gelatine has had time to cool, thus producing a perfect union and adhesion of the two 100 materials. I have found in practice that a duplicating roll or sheet produced by the above process is entirely satisfactory in every respect, the gelatinous composition remaining firmly attached under all ordinary 105 working conditions.

In the accompanying drawings, 3 represents the foundation or backing of a roll or sheet constructed according to my invention, which may be, as above explained, of paper, 110

oilcloth, or any suitable material. 4 represents the adhesive material applied to said backing 3, and 5 represents the layer of gelatinous composition applied thereto.

5. The advantages of my invention will be obvious from what has been above said.

Having thus described my invention, what I claim as new and desire to secure by Letters Patent is as follows:

10. 1. A duplicating roll or sheet adapted for use upon duplicating machines or the like, comprising in combination a backing sheet, a layer of material thereon having a comparatively low melting point, and a layer of material 15 on said first named layer having a comparatively high melting point.

2. A duplicating roll or sheet adapted for use upon duplicating machines or the like, comprising in combination a backing sheet, 20 a layer of gelatinous material having a melting point of about one hundred and fifty degrees Fahrenheit, and a layer of material between said backing sheet and said gelatinous material, having a melting point sub-

25 stantially lower than the melting point of said gelatinous material.

3. A duplicating roll or sheet adapted for use upon duplicating machines or the like, comprising in combination a backing sheet, 30 a layer of material as rubber cement applied thereto, and a layer of gelatinous com-

position applied to said layer of rubber cement.

4. The process of producing a duplicating roll or sheet adapted for use upon duplicating machines or the like which consists in applying to a suitable backing sheet a layer of material having a comparatively low melting point, and applying to said first named layer a layer of material having a 40 comparatively high melting point.

5. The process of producing a duplicating roll or sheet adapted for use upon duplicating machines or the like which consists in applying to a suitable backing sheet a 45 layer of material having a melting point of about one hundred and ten degrees Fahrenheit and applying to said first named layer a layer of material having a melting point of about one hundred and fifty degrees 50 Fahrenheit.

6. The process of producing a duplicating roll or sheet adapted for use upon duplicating machines or the like which consists in applying to a suitable backing sheet a layer of material as rubber cement, and applying to said rubber cement a layer of hot liquid gelatinous composition.

In witness whereof I have hereunto signed my name this 1st day of May 1923.

ALBERT ISAACS.